







tively, the lossy material can be applied to the exterior coat by means of spraying or dipping from a suspension of the lossy material.

The following specific examples illustrate the results achieved employing different variations of the process:

#### EXAMPLE 1

A prime layer of slurry was made up containing 25% by weight graphite particles, the slurry having the following composition:

30% colloidal silica binder  
45% suitably sized zircon flour  
25% suitably sized graphite

After the mold was completely built up, it was subjected to microwave irradiation at a frequency of 2450 mH at a power output of about 7.2 kilowatts. It was found that the mold thus produced was dewaxed in about 3 minutes.

#### EXAMPLE 2

The same type of mold as specified in Example 1 was built up, except that the graphite particles were included in an amount of 25 percent by weight in each of 2 prime layers. Under the same conditions of irradiation as in Example 1, the mold was found to be dewaxed in 2 minutes.

#### EXAMPLE 3

In this example, the first concrete layer was modified by the addition of 25 percent by weight of graphite particles. While the rupture stress of the resulting mold was decreased from that observed in connection with Examples 1 and 2, the dewaxing took place in only 1 minute.

#### EXAMPLE 4

In this example, the first concrete layer consisted of a fifty-fifty mixture of graphite and sand. It was found that under the conditions of dewaxing previously mentioned, the mold assembly could be dewaxed in about 2½ minutes.

#### EXAMPLE 5

In this example, the finished mold was dipped in an aqueous suspension of carbon particles in which the carbon constituted 30 percent by weight of the suspension. Dewaxing under the conditions previously mentioned occurred in 2 minutes.

#### EXAMPLE 6

A finished mold assembly was sprayed with an aqueous suspension containing 15 percent by weight of carbon particles of colloidal size. The mold assembly was dewaxed in approximately 2 minutes under the aforementioned conditions of dewaxing.

#### EXAMPLE 7

In this example, the graphite particles were included in one of the prime coats in a 25 percent concentration by weight. The concrete layer next to the prime coat consisted of a fifty-fifty mixture of carbon particles in sand. It was found that this mold could be dewaxed in about 2 minutes.

The amount of exposure to microwave radiation in order to achieve dewaxing is dependent on at least four factors. These are the configuration of the shell, the

type of lossy additives, the concentration of the additive, and the power level of the microwave source. The use of auxiliary heat following microwave heating was also found to decrease the time of microwave exposure required to about one half. Tests made on production size molds at a power level of 10 kilowatts for 4 to 5 minutes followed by exposure to a hot air oven at 200°F. for an equivalent amount of time showed that such molds could be completely freed of wax.

A continuous furnacing setup for microwave dewaxing is shown in the accompanying drawing. In the drawing, reference numeral 10 indicates generally a table on which the various units are supported, including a metal vestibule 11 into which the mold clusters to be

dewaxed are introduced. The clusters are supported on suitable pallets (not shown) which are received on drive rollers 12 and are driven by a drive chain and sprocket or other suitable driving means located in a housing 13. As the pallets are propelled along the rollers 12, they engage a microswitch or other switch means to actuate a pair of air cylinders 14 and thereby lift a metallic baffle 15 which serves as a shield to prevent the high frequency energy from radiating into the vestibule 11. As the pallet proceeds through the furnace, it engages other switch means (not shown) which deenergizes the air cylinders 14 to lower the baffle 15 into its shielding position and energizes a pair of air cylinders 16 to raise a baffle 17 and thereby permit entry into the microwave treating section. This section is en-

ergized by a pair of microwave generators 18 and 19 which deliver microwave energy through a system of wave guides 20 and 21 at the mold clusters supported on the pallets. The entire system, including the hot air system, trough discharge and the conveyor are under

the control of a control unit 22.

After a predetermined residence time in passing through the microwave section, the molds are passed through a hot air zone in which there is located a blower housing 23 containing a blower 31 which directs hot air at a temperature of about 180° to 190°F. at the mold assembly to remove the last traces of any waxy material contained therein. The movement of the pallet through the hot air zone then actuates another switch (not shown) to energize a pair of air cylinders

24, thereby raising a metal baffle 25 permitting egress from the hot air zone. When the baffle 25 is raised, a succeeding baffle 26 is still in its lowered or shielding position, and after the pallet passes the baffle 25, it energizes still another switch means to deenergize the air cylinders 24 and energizes a pair of air cylinders 27 to raise the baffle 26 and thereby permits the dewaxed mold assembly to be withdrawn from the conveyor at an exit vestibule 28.

The pallets are suitably apertured so that the molten wax drops down into a trough 29 which extends the length of the conveyor from the beginning of the microwave zone to the exit vestibule. A discharge 30 is provided to deliver the recovered waxy material to filtering or other purifying means so that it may be reused in the manufacture of patterns.

The microwave method of pattern removal involves the rapid generation of heat at the optimum place required, at or near the pattern or mold material because of the penetrating power of high frequency radiation.

Heat transfer within the mold is therefore by conduction rather than by a slower combination of convection and/or thermal radiation plus conduction, as in other

65

60

65

60

